

Dec. 27, 1938.

S. CHYLINSKI

2,141,377

PROCESS AND APPARATUS FOR THE PRODUCTION OF SHEETING

Filed July 31, 1936



INVENTOR.  
BY Stanislas Chylinski  
Tomasz Allwibe  
ATTORNEY.

## UNITED STATES PATENT OFFICE

2,141,377

## PROCESS AND APPARATUS FOR THE PRODUCTION OF SHEETING

Stanislas Chylinski, Wilmington, Del., assignor to E. I. du Pont de Nemours &amp; Company, Wilmington, Del., a corporation of Delaware

Application July 31, 1936, Serial No. 93,697

4 Claims. (Cl. 34—24)

This invention relates to web, sheet or film contacting surfaces. More particularly, it relates to such contacting surfaces for the drying of materials in the form of webs, sheets and films. 5 The invention will be described in terms of the drying of non-fibrous sheets and films, such as, regenerated cellulose, although the invention is not to be limited thereto.

In the manufacture of regenerated cellulose sheets and films, a solution such as viscose is brought into pellicular form which is regenerated and purified, and sometimes subjected to a sizing treatment, by passing the same through various treating tanks. After emerging from the last 10 of these tanks, the film is dried by leading it over a series of internally heated rollers, after which it is wound up into mill rolls. In the drying of these films great lateral contraction occurs. A film after it has been dried is often 15 scarcely half the width of the film when it is first formed. Although the sheet and film producing machine readily prevents the film from contracting in the longitudinal direction, by keeping it under a longitudinal tension, special 20 steps must be taken to materially prevent or restrict the film from shrinking laterally.

Great difficulty has been experienced, heretofore, in satisfactorily restricting the lateral shrinkage of sheets and films composed of non-fibrous materials. In an effort to overcome this 30 difficulty, the drying rollers have been provided with an adhesive surface as disclosed in United States Letters Patent to Herndon, No. 2,000,079. The procedure set forth in this patent reduces 35 lateral shrinkage to a great degree but has several defects which this invention is intended to overcome. In the first place, the iron rollers usually serving as a base for the coating applied according to the Herndon patent are only fair 40 conductors of heat, and when a resin, lacquer or varnish coating of the type disclosed by Herndon is applied thereto, the heat conduction of the 45 roller as a whole is still further reduced, due to the low heat conductivity of the coating itself. Molded resin drying rollers, such as disclosed by Herndon, have a still lower heat conductivity 50 than iron or steel coated rollers. Secondly, the character of the surface depends to a great extent upon the quality of the coating applied and the method of application. Variation in coating 55 application technique has resulted in very undesirable film width and quality. Uneven application of coating produces uneven wear which results in unsatisfactory film. Varnish coatings

and the like of the Herndon type are also quite perishable and must be frequently renewed.

Additional difficulties have been encountered in the drying of specially treated film, when subjected to drying on drier roll surfaces coated with 5 varnish or similar composition. Certain types of film are provided with a tenuous coating or size in the last treating tank, such as is disclosed in United States Letters Patent Numbers 2,008,815 and 2,011,246. This size sometimes tends to come 10 off on the drier roll surfaces to a certain extent, and when this has proceeded for a period of time, the accumulation of size on the drier roller causes haziness in the film. When the size is removed from the roller in order to overcome this haziness, some of the coating is also taken off, resulting in non-uniform drier roll surfaces. Because of this, it is necessary to recoat the drier rollers 15 more frequently, thus causing production delays and additional expense. 20

It is therefore an object of this invention to provide an improved surface for drying materials in web form, and particularly non-fibrous, cellulose sheets and films cast from aqueous solutions. 25

It is another object of this invention to provide an improved method for the production of webs, sheets and films, particularly non-fibrous cellulose sheets and films cast from an aqueous solution. 30

It is a further object of this invention to provide an improved method for drying webs, sheets and films involving the restraining of the lateral shrinkage thereof. 35

It is still another object of this invention to provide a better heat conducting surface on drier rollers.

It is still another object of this invention to provide a drier roller surface of the required characteristics which will be more permanent 40 than those known heretofore.

Yet another object of this invention is to provide a drier roll surface of the required characteristics which can be renewed easily and uniformly, and can be precisely duplicated. 45

Other objects of the invention will appear hereinafter.

The objects of the invention are accomplished, in general, by passing wet webs, sheets or films over a drying surface, for example, a drying 50 roller, composed essentially of aluminum on which a layer of aluminum oxide has been formed by means of an electric current.

The details of the invention will be more clearly apparent by reference to the following de- 55

scription taken in connection with the accompanying illustration, in which:

Figure 1 is a vertical sectional view, showing a drying roller constructed in accordance with the present invention.

Figure 2 is a diagrammatic elevational view showing an apparatus suitable for use in the production of non-fibrous cellulosic sheets or films.

It is known that an aluminum body may be given an electrolytic treatment to form thereon a comparatively hard, inert aluminum oxide surface. The aluminum body, which may be formed by drawing, rolling, casting or any other desired manner, is first evened by a suitable machining operation. It is also preferably further smoothed by a grinding, burnishing or buffering operation. However, in some cases it may be desired to form a slightly roughened surface on the machined body. Desirable roughened surfaces may be obtained by sand blasting with sand of various degrees of fineness or by etching with an etching solution, for example, by subjecting the aluminum body to an aqueous solution containing 5% caustic soda and 4% sodium chloride at a temperature of 77° C. Any other method of uniformly roughing the body may be equally applicable.

After the aluminum body has been suitably smoothed or roughened, as the case may be, it is placed into an electrolytic bath through which an electric current is passed, and in which the aluminum body serves as the anode of an electrolytic cell. This treatment causes the surface of the body to be changed to an aluminum oxide, the depth of the oxide surface being dependent upon the specific procedure employed and length of time of the operation. This treatment will be referred to hereinafter as "anodizing".

Referring to Figure 1 of the drawing, reference 40 to character 11, designates a drying roller of the type commonly used in the production of transparent regenerated cellulose pellicles. The drying roller 11 may be suitably mounted in bearings 13 and 15 and is provided with an open end 45 17 through which a liquid heating medium may be circulated within the roller 11. The heating medium may be introduced into the interior of the roller 11 by means of conduit 19 which is preferably provided with a plurality of apertures 21 for the even distribution of the liquid. The heating liquid flows from the roller 11 through the open end 17 and is withdrawn through the funnel-shaped conduit 23 to be reheated and again re-circulated through the roller 50 55 11 in a known manner. The heating liquid is ordinarily water, although any other liquid or gaseous heating medium may be utilized. The roller 11 is provided at the external surface thereof with an aluminum oxide coating 25 prepared 60 thereon by anodization through means of an electric current. This external surface 25 readily conducts the heat from the aluminum roller 11, which in turn is heated by the heating medium passed against the internal surface thereof. Due 65 to the high heat conductivity of aluminum, the heat is rapidly and efficiently conducted to the anodized aluminum oxide surface 25, and wet webs, films or sheets placed in contact with the hot roller surface 25 are effectively dried in a 70 minimum period of time by contact with a relatively small number of such drier roller surfaces.

Figure 2 diagrammatically illustrates the extrusion of a non-fibrous cellulosic material into a coagulating bath 50 by means of an extrusion device generally indicated by 52. The film as it

passes from the extrusion device 52 is coagulated in the bath 50 and is thence passed through a series of washing and purifying baths (not shown), and in some cases through a sizing bath 54 from which it is removed to be passed into drier 56 in which are positioned a series of drier rollers 11. The drier 56 may be provided with a covering 58 to form a chamber from which the moist air may be removed through outlet 60. It may, in some cases, however, be desired to dispense with the cover 58 and merely allow the moist atmosphere driven off from the film to pass into the surrounding atmosphere. After passing through the drier or rather over the drier rolls 11, the web, sheet or film 10 is wound into a mill 15 roll 62 in a known manner.

The following specific example is given to illustrate in detail one method in which the anodizing of an aluminum body may be carried out. However, the invention is not to be limited thereto.

An aluminum body, drawn into hollow cylindrical roller form and suitably machined and buffed, is placed in a lead lined tank containing a 15% solution of sulphuric acid at a temperature of 68° to 72° F. The aluminum roll is made 25 to constitute the anode, and the lead lining in the tank the cathode of an electrolyzing circuit, through which a current of about 18 amperes per square foot of aluminum is passed. The aluminum roll is electrolyzed in this manner for a 30 period of about 50 minutes, at the end of which time the surface of the aluminum is converted to an oxide approximatey 0.001 inch deep. The body is then washed and is ready for any further treatment to which it is desired to subject the 35 same.

In recent years, there has been developed an improved method for after-treating anodized aluminum surfaces. This method is known as "sealing", and consists in placing the anodized 40 aluminum, after washing, in boiling water, where it remains for a suitable period of time, for example, thirty minutes. The sealing operation has the effect of giving to the oxide surface a high polish and making it denser, more impervious to 45 certain liquids and less sticky in character. It is thought that this is due to the fact that, before sealing, the surface apparently consists of pointed serrations, the points of which are quite widely separated, and that, after sealing, these points 50 appear to be drawn closer together. This may have some distinct bearing on the stickiness of the unsealed anodized surfaces above referred to.

The term "sealed" as used throughout the present specification and claims refers to surfaces 55 which have been treated as outlined in the preceding paragraph. Contrarywise, the term "unsealed" refers to surfaces which have not been so treated.

Although an anodized and sealed aluminum 60 surface may in some cases be very desirable due to its smoothness and highly efficient conduction of heat, it offers no substantial improvement over previously known drying rollers in preventing or reducing transverse shrinkage of sheets and films. 65 This may possibly be due to the fact that the sealing treatment apparently saturates the surface with water of hydration. When it is not saturated, the water contained in the film being dried may have sufficient chemical affinity for the aluminum oxide to restrain shrinkage of the film.

The remarkable discovery has been made, however, that by omitting the sealing treatment, anodized aluminum surfaces are extremely efficient in preventing transverse shrinkage of 75

webs, sheets and films during the drying thereof. Drying rollers provided with an anodized, unsealed surface, therefore, are found to have great utility, not only in reducing the shrinkage of sheets or films to one-half or less than one-half as previously obtainable, but also in procuring accurate control of the lateral shrinkage of such sheets and films.

In view of the efficacy of unsealed anodized aluminum surfaces in the prevention or restriction of lateral shrinkage in non-fibrous cellulosic sheets and films, it might be expected that this characteristic of anodized aluminum surfaces might be enhanced by submitting such surfaces prior to the anodization thereof to a roughening treatment such as by sand blasting, rough grinding or the like. It has been found, however, contrary to expectations, that the efficacy of the special aluminum oxide surface in preventing shrinkage of film dried thereon is materially improved by making the surface as smooth as possible before forming the oxide surface thereon. This is possibly due to the fact that the particular aluminum oxide surface is the effective means for preventing shrinkage, and the greatest conversion to the oxide and the greatest contact of the oxide with the film being dried will be effected by leveling off of the high points of the rough surface prior to its conversion to the oxide. This is preferably effected by machining, and further enhanced by buffering.

Another peculiar characteristic of this anodized and unsealed surface and its effectiveness in preventing shrinkage is its greater efficiency or effectiveness when in contact with wet film. Tests have been made to determine the behaviour of regenerated cellulose films of varying moisture content, dried on such a surface. It has been found that this surface although very effective when the film is wet, becomes much less effective as it approaches dryness. For example, a film containing less than approximately 70% water, based on the weight of the cellulose, is not prevented from shrinking during the drying thereof to any greater extent than by a surface of the type disclosed in U. S. Patent Number 2,000,079. This characteristic of unsealed anodized surfaces is very desirable. The greatest amount of shrinkage of non-fibrous cellulosic sheets and films occurs above the 70% moisture content of sheets and films, and it is this shrinkage which it is usually desired to prevent, in order to secure a film of maximum width. The shrinkage occurring below the 70% moisture content is known as "permanent shrinkage" and it is usually desired to permit this shrinkage to take place.

It is not definitely known why an unsealed anodized aluminum surface will have a greater efficiency to prevent shrinkage of films when they are wet, however, it is believed that this may be due to the great affinity of aluminum oxide for water. Since water is intimately bound in the structure of a gel regenerated cellulose film, it is possible that as the film is brought into contact with the aluminum oxide surface of the roller, the water in the film will form a physico-chemical union with the aluminum oxide roller surface, thus restraining the film from shrinking. As the drying proceeds, less water is available for forming the union between the film and the roller surface and the restraining force thus becomes weaker.

In view of the above described unusual but

desirable characteristics of unsealed, anodized aluminum surfaces, it is ordinarily preferred that the aluminum body is not subjected to a sealing treatment after anodization. Nevertheless, in certain cases, where shrinkage of sheets and films is unimportant, or in cases where such shrinkage is desirable, it may be desired to use a sealed anodized aluminum surface in view of its greater smoothness and high heat conductivity. The type of anodized roll surface may be varied in different parts of the same machine, or for the production of different types of film in different machines according to the shrinkage effects desired.

Various other finishing treatments may be applied to anodized aluminum surfaces. Anodized drying roller surfaces for use in drying certain special types of film may require the application of certain finishing materials to the roller surface. In some cases it has been found desirable, for example, that rosin or silica be applied to an anodized aluminum surface which is to be used as a drying surface. Rosin may, for example, be applied thereto from solution or in molten or powdered form. The silica may be applied to such a surface by dipping the surface for ten minutes in a 10% solution of sodium silicate.

The following table illustrates the effectiveness of drying roller surfaces in restraining the transverse or lateral shrinkage of regenerated cellulose pellicles. The table gives the result of tests performed on sealed and unsealed, roughened and smoothed anodized drying roller surfaces as well as previously known drying roller surfaces. In the first column is listed the various types of drying roller surfaces tested. In the second column is shown the average amount of shrinkage occurring during the drying step, in percentage of the width of the pellicle emerging from the final liquid treating bath. In the third column is shown the amount of variation in shrinkage that would occur in films dried on the various surfaces (probable error or reliability tolerance). It will be noted that in all cases the anodized aluminum surfaces show much greater controllability of shrinkage than previously known surfaces.

Table

| Description of surface                                  | Shrinkage | Tolerance | 50      |
|---------------------------------------------------------|-----------|-----------|---------|
|                                                         |           |           | Percent |
| <i>Aluminum</i>                                         |           |           |         |
| Machined, buffed, anodized, not sealed                  | 5.39      | ±0.14     |         |
| Machined, anodized, not sealed                          | 7.34      | ±0.33     | 55      |
| Machined, anodized, impregnated with silica             | 12.42     | ±0.46     |         |
| Etched 5 minutes, anodized, sealed                      | 21.55     | ±1.08     |         |
| Etched 3 minutes, anodized, sealed                      | 23.90     | ±0.64     |         |
| Very fine sand blast, anodized, impregnated with silica | 31.08     | ±0.18     |         |
| Very fine sand blast, anodized, sealed                  | 33.83     | ±0.36     |         |
| Etched 10 minutes, anodized, sealed                     | 35.40     | ±0.74     | 60      |
| Fine sand blast, anodized, sealed                       | 37.39     | ±0.68     |         |
| <i>Non-aluminum</i>                                     |           |           |         |
| Lacquered, rubber covered cast iron                     | 15.23     | ±3.28     |         |
| Varnished steel (U. S. Patent 2,030,079)                | 15.53     | ±1.12     | 65      |

The term "aluminum" in this specification and claims is intended to include alloys where aluminum is the essential alloying element, normally comprising at least 75% to 90% of the alloy. Generally speaking, the qualities sought for in an alloy are hardness and ease and effectiveness of anodization. The former, as is known, is effected by adding to aluminum one or more of certain elements, such as magnesium, chromium, silicon, copper, zinc, manganese and nickel. It is true, 70

however, that these alloying elements or hardeners deleteriously affect to a greater or lesser extent ease and effectiveness of anodization. A compromise, therefore, is sought for between 5 hardness and anodization. An alloy which has been found very effective is one containing one and one-quarter per cent magnesium, one-quarter per cent chromium, .7% silicon and the remainder aluminum.

10 Heretofore, the principal advantage of anodized aluminum surfaces was thought to be their hardness and inertness. It has now been found, however, that due to certain peculiar characteristics 15 of these surfaces, they are found to be very advantageous for use in the preparation of webs, sheets and films in which it is desired to prevent or restrain lateral shrinkage thereof. Drier rollers constructed of aluminum and provided with an anodized aluminum surface are found to be 20 light in weight, easy to handle and provide greatly improved heat transfer. When the surface becomes worn down, it can be reproduced easily, cheaply, efficiently and accurately. Undesirable 25 variations in reproducing the anodized surfaces can be easily avoided, and thus uniform surfaces will exist throughout the various sheet and film producing machines. The accurate reproducibility of the anodized surfaces and the close controllability of shrinkage effects in film dried on 30 such surfaces may make it desirable to use this invention whether or not shrinkage is allowed to take place.

The wearing qualities of the anodized aluminum surfaces are such that they will need to be 35 renewed much less often than those produced in accordance with U. S. Patent No. 2,000,079. Due to the hardness of anodized aluminum surface it has been found to be particularly desirable in 40 resisting abrasion by knife cuts which are frequently made on sheets and films traveling over the rolls. If, by drawing a knife over a drier roller surface, it were abraded to the extent that a burr was raised thereon, it would be entirely 45 unsatisfactory for the further production of cellulose film. Anodized aluminum surfaces have the property of resisting abrasion by knife cuts to the extent that no burr will be raised on the surfaces thereby.

Another advantage of anodized aluminum drying rolls comprises the ease with which sizing materials may be removed therefrom. When a sizing solution accumulates upon the rollers to such an objectionable extent that it causes haze 5 in the film, it can be easily and quickly removed by means of solvents without injuring the roll surface. Finally, in the preferred embodiment 10 of this invention, in which the anodized aluminum surfaces have not been subjected to a sealing treatment, lateral or transverse shrinkage in the film is removed to one-half or one-third of that known heretofore.

While the invention has been described in terms of the drying of films of regenerated cellulose, it 15 is to be understood that it is equally applicable to the drying of other materials in pellicular form, such as other non-fibrous materials, including cellulose esters and ethers, gelatin and casein as well as fibrous sheet material such as paper and 20 the like. It is also applicable to the prevention of shrinkage in sheets and films during other steps in the manufacture thereof which involve contact with a moist or wet sheet or film.

It is obvious that various changes and modifications may be made in the process and apparatus hereinabove described without departing from the nature and spirit of the invention. It is therefore, to be understood that the invention is not to be limited except as set forth in the following appended claims.

I claim:

1. In the production of non-fibrous cellulosic pellicles, the step which comprises drying said pellicles by passing the same over a heated un- 35 sealed anodized aluminum surface.
2. In the production of non-fibrous cellulosic pellicles, the step which comprises drying said pellicles by passing the same over a heated smoothed and unsealed anodized aluminum sur- 40 face.
3. The method of claim 1 characterized in that the pellicles are regenerated cellulose pellicles.
4. The method of claim 2 characterized in that the pellicles are regenerated cellulose pellicles. 45

STANISLAS CHYLINSKI.